

# UNITED STATES PATENT OFFICE.

MOSES G. FARMER, OF SALEM, MASSACHUSETTS.

## IMPROVED ALLOY OF ALUMINUM.

Specification forming part of Letters Patent No. 44,086, dated September 6, 1864

*To all whom it may concern:*

Be it known that I, MOSES G. FARMER, of Salem, in the county of Essex and State of Massachusetts, have invented an Improved Aluminum Alloy; and I do hereby declare that the following is a description of my invention sufficient to enable those skilled in the art to practice it.

In the United States Letters Patent No. 38,301, granted to me April 28, 1863, for improved alloys of aluminum, I therein described alloys in which the proportion of copper varied from eighty to ninety-eight per cent. of the whole alloy, and in which the aluminum and other light-colored metals formed from twenty to two per cent. of the whole alloy, the proportion of the aluminum to the whole quantity of light-colored metals used varying from ten to ninety-five per cent.

My present invention consists of an alloy not within the range of those included in my said patent. Said alloy is useful in that, among other uses, it is particularly adapted for formation into and for use as nails; and it consists in a mixture in which the copper therein may vary from sixty-five to eighty per cent. of the whole, and the light-colored metals

therein from thirty-five to twenty per cent. of the whole, the aluminum being from three-tenths to three-thousandths of the whole quantity of the light-colored metals used. By preference I employ for the light-colored metals other than the aluminum-named steel, iron, zinc, tin, nickel, antimony, or arsenic, either separately or in any desired combination with reference to such peculiar quality as I may desire to obtain for any special purpose. For example, a peculiarly tough and ductile alloy results from making up the whole quantity of the light-colored metals in the following proportions, viz: ninety-one and six-tenths per cent. of zinc, six and seven-tenths per cent. of cast-steel, one and seven-tenths per cent. of aluminum.

I claim—

The alloy compounded of the metals and in the proportion substantially as specified.

In witness whereof I have hereunto set my hand this 19th day of April, A. D. 1864.

MOSES G. FARMER.

In presence of—

J. B. CROSBY,  
F. GOULD.